

# United States Patent

Gonzales et al.

[15] 3,645,667

[45] Feb. 29, 1972

[54] **NONAQUEOUS CROSS LINKING OF  
CELLULOSE WITH A METHYLOLATED  
UREA IN THE ABSENCE OF AN ACIDIC  
CATALYST**

[72] Inventors: **Elwood J. Gonzales**, Gretna; **Ralph J. Berni**, Metairie; **Ruth R. Benerito**, New Orleans, all of La.

[73] Assignee: **The United States of America as represented by the Secretary of Agriculture**

[22] Filed: **May 22, 1970**

[21] Appl. No.: **39,922**

[52] U.S. Cl.....**8/116.3**, 8/116.2, 117/139.4

[51] Int. Cl.....**D06m 13/14**, D06m 13/16, D06m 13/38

[58] Field of Search.....**8/116.3**, 116.2

[56] **References Cited**

UNITED STATES PATENTS

|           |         |                |                      |
|-----------|---------|----------------|----------------------|
| 3,533,728 | 10/1970 | Shippee et al. | ..... <b>8/116.3</b> |
| 3,434,794 | 3/1969  | Tovey          | ..... <b>8/116.3</b> |
| 3,046,079 | 7/1962  | Reeves et al.  | ..... <b>8/116.3</b> |
| 2,208,632 | 7/1940  | Dreyfus        | ..... <b>8/116.3</b> |

|           |        |                |                      |
|-----------|--------|----------------|----------------------|
| 2,588,640 | 3/1952 | Lehmann et al. | ..... <b>8/116.3</b> |
| 3,043,719 | 7/1962 | Burr et al.    | ..... <b>8/116.3</b> |
| 3,090,665 | 5/1963 | Parsons et al. | ..... <b>8/116.3</b> |
| 3,183,054 | 5/1965 | Fischer et al. | ..... <b>8/116.4</b> |

OTHER PUBLICATIONS

Chance et al., American Dyestuff Reporter, Vol. 51, No. 16, pp. 28-32, August 6, 1962.

Porter et al., Textile Research Journal, 35, pp. 159-167 (1965).

*Primary Examiner*—George F. Lesmes

*Assistant Examiner*—J. Cannon

*Attorney*—R. Hoffman and W. Bier

[57] **ABSTRACT**

This invention comprises the treatment of cellulosic textiles in the absence of an acidic catalyst with dimethylolethyleneurea (DMEU) dissolved in nonaqueous or predominantly nonaqueous solvent systems, such as neat dimethylformamide, neat dimethylacetamide, 90 percent (vol.) ethanol in water, 90 percent (vol.) dioxane in water, 90 percent (vol.) tetrahydrofuran in water, and 50 percent (vol.) dimethylformamide in dioxane. The cellulosic products thus modified have high dry and wet wrinkle recovery when compared to cellulosic textiles treated with DMEU dissolved in water only.

5 Claims, No Drawings

**NONAQUEOUS CROSS LINKING OF CELLULOSE WITH  
A METHYLOLATED UREA IN THE ABSENCE OF AN  
ACIDIC CATALYST**

A nonexclusive, irrevocable, royalty-free license in the invention herein described, throughout the world for all purposes of the United States Government, with the power to grant sublicenses for such purposes, is hereby granted to the Government of the United States of America.

This invention relates to the treatment of cellulosic textiles with dimethylolethyleneurea (DMEU) dissolved in nonaqueous or essentially nonaqueous solvents without added external catalyst to impart wash-wear properties to cellulosic materials. This type of system should find use in decreasing water pollution since the organic or nonaqueous component may be reclaimed or used over again in the textile treating process. From the standpoint of economics, such as reclamation of the organic portion of the solvent system should ultimately decrease the cost of the process.

The main object of the instant invention is to provide a process wherein enhanced dry and wet creases recovery may be imparted to cellulosic textiles in which no external added catalyst is needed.

A second object of the instant invention is to apply the process to cellulosic textile from nonaqueous to predominantly nonaqueous solvent systems.

A third object of the instant invention is to react the DMEU with the cellulosic textiles at an elevated temperature—about 160° C.—only without prior drying at lower temperature—about 60° C.

To those skilled in the art it is well known that aqueous solutions of DMEU and other nitrogenous resins must be reacted with cellulosic textiles in the presence of added Lewis-type catalysts, such as acids and metal salts, to impart desirable wash-wear properties to the finished fabric or garment. Ziifle, et al., (Textile Research Journal 31, No. 4, pp. 349-365, 1962), have applied DMEU to cotton cellulose in the presence of metal salt catalysts, such as MgCl<sub>2</sub>, Mg(NO<sub>3</sub>)<sub>2</sub>, ZnCl<sub>2</sub>, and Zn(NO<sub>3</sub>)<sub>2</sub> to obtain enhanced dry and wet crease recovery properties. In accordance with the main object of the instant invention described above, we require no added Lewis-type catalyst to effect reaction with the cellulosic materials to obtain the desirable wash-wear properties. Ziifle, et al., also applied DMEU to cotton cellulose from all-aqueous solutions. In accordance with the second object of the instant invention described above, one invention requires nonaqueous or predominantly nonaqueous solvents. In accordance with the third object of the instant invention described above, we reacted DMEU with the cellulosic textiles at an elevated temperature with one heating, whereas the prior art required a preliminary drying step at about 60° C. prior to curing at an elevated temperature, in order to achieve the desirable wash-wear properties.

The impregnation of the cellulosic material is generally carried out in this manner. The material is immersed in neat

then submitted to a cure at about 160° C. for about three minutes. For the process of this invention, it is not necessary to add a catalyst for the purpose of obtaining wrinkle recovery properties on the textile.

5 The materials to which our invention can be applied include cotton, rayon, ramie, jute, flax, and the like, and in the case of cotton we have specifically applied our invention to the textile in the form of woven fabrics with satisfactory results. Those skilled in the art can readily visualize the extension of this application to other forms of textiles in the realm of cellulosic materials.

10 The following examples are presented to illustrate the invention, and since procedure and conditions can be varied by those skilled in the art, the examples are not set forth to establish any particular limits.

15 The treated cotton fabrics were submitted to selected standard tests as well as the other tests indicated here. Breaking strength determinations were done by the ASTM Method D39-49; dry wrinkle recovery determinations were done by

20 the ASTM Method D1295-60T; flex abrasion (bar 575) values were obtained by the ASTM Method D1175-64T; and wet wrinkle recovery determinations were done by the Lawrence and Phillips method described in American Dyestuff Reporter, vol. 45, P. 548-550, 561 (1956). Nitrogen values were obtained by the Kjeldahl Method; and formaldehyde values were obtained by the chromotropic acid method.

**EXAMPLE 1**

30 A sample of cotton printcloth (80 × 80 thread count) weighing about from 9 to 10 grams was impregnated with a 0.55 molar solution of DMEU in neat DMF and padded twice through a laboratory wringer to obtain approximately 90 percent wet weight pickup. The sample was cured in a forced-air oven three minutes at about 160° C. The sample was then washed 15 minutes in hot running tap water (pH = 9-10) and allowed to equilibrate in the laboratory under ambient conditions. 35 The treated sample was then submitted to select evaluation, as described earlier in the specification, and the desired and notable properties together with the results of chemical analyses were recorded. The treated fabric had a 6.8 percent weight gain, 2.04 percent nitrogen, 2.2 percent formaldehyde, 77 percent retention of breaking strength (warp), 276 cycles flex abrasion (bar 575). The dry crease recovery (W+F)<sup>o</sup> was 270; the wet crease recovery (W×F)<sup>o</sup> was 252. Another piece of 80 × 80 cotton printcloth similarly treated with 0.55 molar solution of DMEU in water gave the following properties: 3.1 percent weight gain, 0.88 percent nitrogen, 1.64 percent formaldehyde, 92 percent retention of breaking strength (warp), 40 308 cycles flex abrasion (bar 575) and only 198 degrees (W+F) dry and 206 degrees (W+F) wet crease recovery.

45 Other examples are given in Table I with their properties.

TABLE I.—PROPERTIES OF COTTON PRINTCLOTH TREATED WITH 0.55 MOLAR DIMETHYLOLETHYLENEUREA (DMEU) IN VARIOUS SOLVENT SYSTEMS

| Example | Solvent system                      | Weight gain, percent | N, percent | HCHO, percent | Ret. brk. str. (w.) percent | Flex abras. cycles | Wrinkle recovery (W+F) <sup>o</sup> |     |
|---------|-------------------------------------|----------------------|------------|---------------|-----------------------------|--------------------|-------------------------------------|-----|
|         |                                     |                      |            |               |                             |                    | Dry                                 | Wet |
| 1.      | Neat DMF                            | 6.8                  | 2.04       | 2.20          | 77                          | 276                | 270                                 | 252 |
| 2.      | Neat DMAc                           | 3.4                  | 1.44       | 1.68          | 86                          | 362                | 232                                 | 185 |
| 3.      | 90% (vol.) ethanol-10% (vol.) water | 6.1                  | 1.65       | 2.19          | 73                          | 373                | 255                                 | 211 |
| 4.      | 90% (vol.) dioxane-10% (vol.) water | 7.1                  | 1.63       | 2.51          | 81                          | 302                | 271                                 | 245 |
| 5.      | 90% (vol.) THF-10% (vol.) water     | 7.1                  | 1.81       | 0.98          | 68                          | 252                | 249                                 | 234 |
| 6.      | 50% (vol.) DMF-50% (vol.) dioxane   | 4.1                  | 1.08       | 1.69          | 78                          | 207                | 233                                 | 205 |
|         | Water                               | 3.1                  | 0.88       | 1.64          | 92                          | 208                | 198                                 | 206 |
|         | Untreated control                   |                      |            |               | (*)                         | 900                | 176                                 | 138 |

\*50 pounds.

dimethylformamide (DMF), 90 percent (vol.) ethanol in water, 90 percent (vol.) dioxane in water, 90 percent (vol.) tetrahydrofuran (THF) in water, neat dimethylacetamide (DMAc), or 50 percent (vol.) DMF in dioxane. The treating bath is also about 0.55 molar concentration in DMEU. Once 75 the material has been impregnated from the treating bath, it is

What is claimed is:

1. A process for imparting high dry and wet wrinkle recovery properties to a cellulosic textile, comprising:
  - a. impregnating the cellulosic textile with a solution consisting of about 0.55 mole of dimethylolethyleneurea per

- liter of solution wherein the solvent is a member selected from the group consisting of 90 percent by volume of ethanol in water, 90 percent, by volume of dioxane in water, 90 percent by volume of tetrahydrofuran in water, and 50 percent by volume of dimethylformamide in dioxane;
- b. removing excess solution from the impregnated cellulosic textile of step (a) until a wet-pickup of about 90 percent by weight, based on the weight of the textile is obtained; and
- c. curing the impregnated textile from step (b) for about

three minutes at about 160°C.

2. The process of claim 1 wherein the solvent is 90 percent by volume of ethanol in water.
3. The process of claim 1 wherein the solvent is 90 percent by volume of dioxane in water.
4. The process of claim 1 wherein the solvent is 90 percent by volume of tetrahydrofuran in water.
5. The process of claim 1 wherein the solvent is 50 percent by volume of dimethylformamide in dioxane.

\* \* \* \* \*

15

20

25

30

35

40

45

50

55

60

65

70

75